# EUROPEAN PATENT SPECIFICATION

(11) **EP 0 671 655 B1**
(45) Date of publication and mention of the grant of the patent: **21.06.2000**
(21) Application number: 95103145.9
(22) Date of filing: 06.03.1995
(51) Int. Cl.: G03C 1/30

(54) **Improved hardening of hydrophylic colloids with imidazolium and triazine combinations**
Verbesserte Härtung hydrophiler Kolloide mit Imidazolium/Triazinkombinationen
Durcissement amélioré de colloids hydrophyliques à l'aide de combinaisons imidazolium/triazine

(30) Priority: 11.03.1994 US 208778
(43) Date of publication of application: 13.09.1995
(73) Proprietor: AGFA-GEVAERT N.V., 2640 Mortsel (BE)
(72) Inventor: Fodor, Ludovic, Hendersonville, North Carolina 28792 (US); Jones, Richard R.M., Hendersonville, North Carolina 28739 (US); Rueger, Reinhold, D-63322 Roedermark (DE); Weberg, Rolf Thomas, Brevard, North Carolina 28712 (US); Weatherill, Timothy Donald, Wilmington, Delaware 19803 (US)
(74) Representative: Ramon, Charles Lucien

(56) References cited:
- EP-A- 0 519 329
- US-A- 3 288 775
- US-A- 3 325 287
- US-A- 5 378 842
- DATABASE WPI Section Ch, Week 8829 Derwent Publications Ltd., London, GB; Class A89, AN 88-200270 & JP-A-63 135 935 (KONICA KK) , 8 June 1988

## Description

### FIELD OF INVENTION

This invention is related to improved hardeners for proteinaceous materials. More specifically this invention is related to a combination of imidazolium and triazine hardeners for crosslinking a proteinaceous material in a photographic film.

### BACKGROUND OF THE INVENTION

Proteinaceous materials are used for a wide variety of applications. One of the predominant useful properties is their ability to swell in aqueous solutions and yet form a solid matrix which is permeable to aqueous solutions upon drying. These properties have been exploited for many generations in the field of photographic sciences and proteinaceous materials are still widely used as a binder for harbouring silver halide grains in the photosensitive layer of photographic films.

Formation of a solid matrix is typically considered to be a result of inter-and intra-molecular hydrogen bonding within both the helical and random regions of proteinaceous materials. If only the natural hydrogen bonding is employed the strength of the matrix is typically insufficient for use in a photographic film. Therefore, it is common practice to add a hardener, also known as crosslinking agent, to a proteinaceous material when used for photographic layers.

Hardeners are chosen, in part, for their ability to link one group on a proteinaceous molecule with another group on the same, or different, proteinaceous molecule. The linking generates a three dimensional network of proteinaceous material. This three-dimensional network has sufficient strength to safely harbour a silver halide grain. Another important aspect of the three dimensional network is an ability to allow solution to permeate freely during the photographic processing steps of development, fix (or bleach) and wash. It is imperative that the solution which freely permeates the matrix is not strongly absorbed. This is particularly important for photosensitive elements since they must often be capable of transiting the photographic processing steps of development, fix, wash and dry in 20-120 sec.

Crosslinking of a binder matrix most often involves the carboxyl groups, amine groups, or combinations thereof. The number of carboxyl groups is substantially larger than the number of amine groups in most commercially available gelatin. Traditional hardeners, such as triazines, described, for example, in US-A-3 288 775 or US-A-3 325 287, are widely accepted as capable of combining amine groups and are thus termed amine-amine crosslinkers. Amine-amine crosslinkers provide a very strong matrix yet the carboxyls are largely unaffected. The unreacted carboxyl groups are deleterious since they strongly absorb processing solution and increase the time required to remove the absorbed solution. The result is an increase in the time and/or energy required for transiting the photographic processing steps identified above. Peptide couplers, such as imidazoliums, described, for example, in JP-A-63 135 935 or EP-A-519 329 are widely accepted as combining a carboxyl group with an amine group to form an amide linkage between binder strands. This is advantageous since the number of free carboxyls is decreased. Unfortunatly, the strength of the peptide-coupled binder is insufficient to transit a processor and total binder destruction is frequently observed.

There has been a long felt need in the art to provide a method of crosslinking a binder which has the strength of an amine-amine crosslinked matrix and the permeability and low solution retention of a binder crosslinked by amide linkages.

An important consideration in crosslinking a binder is the pH of activity. This is particularly important when comparing amine-amine crosslinking reactions with reactions that form amide linkages. Amine-amine crosslinkers, like triazines, are typically stable around a neutral pH (∼7) and decomposition, or decreased reactivity, is observed above or below neutrality. Peptide couplers, especially imidazoliums, are susceptible to instablility at higher pH and decomposition is accelerated above a pH of approximately 6.2. Therefore, if a pH is employed for optimum amine-amine crosslinking, the decomposition of imidazolium complexes is in competition with crosslinking reactivity. If a pH is employed which is suitable for formation of amide linkages by an imidazolium the amine-amine crosslinking reagents become unstable in solution. At intermediate ranges neither crosslinking method is efficient. Partly due to the stability differences, skilled artisans have considered imidazolium type coupling agents, and amine-amine coupling agents to be incompatable since a suitable solution pH was unavailable. By methods described herein the advantages of imidazoliurn couplers and amine-amine couplers can be used concurrently to provide a strong matrix with low water absorption.

### SUMMARY OF THE INVENTION

It is an object of the present invention to provide a process for forming a photographic element involving a hardening combination which effectively increases the strength of the matrix.

It is another object of the present invention to provide a process involving a hardening combination which decreases the amount of fluid absorbed and restrained during processing.

A particular feature of the present invention is the ability to provide a photographic element which has a strong matrix, low fluid absorption and can undergo photographic development without detrimental effects.

These and other advantages, as will be apparent from the description, are provided in a process for forming a photographic element comprising the steps of:
forming at least one liquid photographic emulsion in at least one storage vessel wherein said liquid photographic emulsion comprises silver halide, hydrophilic colloid and a solvent;
transporting said liquid photographic emulsion to an interface region;
adding at least one compound I as defined below and at least one compound II as defined below;
mixing said liquid photographic emulsion with said compound I and said compound II thereby forming a coating solution;
transporting said coating solution to a coater;
coating said coating solution on a substrate thereby forming a liquid layer;
removing said solvent from said liquid layer to form a dry coated layer,
wherein the time between addition of the hardeners and coating is not so long that crosslinking and decomposition begin to occur;
compound I is a compound of Formula I: wherein:
- Y¹: is an alkyl, or substituted alkyl, of 1 to 24 carbons; aryl, or substituted aryl, of 6 to 24 carbons; aralkyl or substituted aralkyl of 7 to 25 carbons; the atoms chosen from C, N, O, and S necessary to form a substituted or unsubstituted 5- or 6-membered ring; -L¹CR⁸CH₂, or a polymer thereof; -C(Y⁴)E; or
- E: is an alkyl, or substituted alkyl, of 1 to 24 carbons; aryl, or substituted aryl, of 6 to 24 carbons; aralkyl or substituted aralkyl of 7 to 25 carbons; -OR⁹; -CN; the atoms chosen from C, N, O, and S necessary to form a substituted or unsubstituted 5- or 6-membered ring;
- L¹: is a linking group;
- R¹: is hydrogen; alkyl, or substituted alkyl, of 1 to 24 carbons; aryl, or substituted aryl, of 6 to 24 carbons; aralkyl, or substituted aralkyl, of 7 to 25 carbons; -OR¹⁰; halogen; nitro, carboxyl, mercapto; alkylamino or substituted alkylamino of 1 to 24 carbons; the atoms chosen from C, N, O, and S necessary to form a substituted or unsubstituted 5-or 6-membered ring;
- R² and R³: independently represent hydrogen; alkyl, or substituted alkyl, of 1 to 24 carbons; aryl, or substituted aryl, of 6 to 24 carbons; aralkyl, or substituted aralkyl, of 7 to 25 carbons; R² and R³ independently may represent, or be taken together to represent, the atoms chosen form C, N, O and S necessary to form a 5- or 6-membered ring;
- R⁴ and R⁵: independently represent hydrogen; alkyl, or substituted alkyl, of 1 to 24 carbons; aryl or substituted aryl of 6 to 24 carbons; aralkyl or substituted aralkyl of 7 to 25 carbons; nitro; carboxyl; mercapto; -OR¹¹; halogen; alkylamino or substituted alkylamino of 1 to 24 carbons ;the atoms chosen from C, N, O, and S necessary to form a substituted or unsubstituted 5- or 6-membered ring;
- R⁴ and R⁵: may be taken together to represent the atoms chosen from C, N, O, and S necessary to form a substituted or unsubstituted 5- or 6-membered ring;
- X⁻: is a counterion;
- Y², Y³ and Y⁴: independently represent O or S;
- R⁶ and R⁷: independently represent hydrogen; alkyl, or substituted alkyl, of 1 to 24 carbons; aryl, or substituted aryl, of 6 to 24 carbons; aralkyl, or substituted aralkyl, of 7 to 25 carbons; the atoms chosen from C, N, O and S necessary to form a substituted or unsubstituted 5- or 6-membered ring;
- R⁶ and R⁷: may be taken together to represent the atoms chosen from C, N, O and S necessary to form a substituted or unsubstituted 5- or 6-member ring;
- R⁸: represents a hydrogen; an alkyl, or substituted alkyl, of 1 to 24 carbons; -C(O)R²⁸; -CN; aryl or substituted aryl of 6 to 24 carbons;
- R⁹: represents hydrogen; alkyl or substituted alkyl of 1 to 24 carbons; aryl of substituted aryl of 6 to 24 carbons;
- R¹⁰ and R¹¹: independently represent hydrogen, an alkyl, or substituted alkyl, of 1 to 5 carbons;
- R²⁸: represents hydrogen; alkyl or substituted alkyl of 1 to 24 carbons; alkoxy or substituted alkoxy of 1 to 24 carbons; amine; alkylamine or substituted alkylamine of 1 to 24 carbons;
and compound II is a compound of Formula II: wherein:
at least two of R¹², R¹³ and R¹⁴ are independently chosen from the groups represented by halogen, preferably Cl or Br; one of
- R¹², R¹³ or R¹⁴: may represent hydrogen; alkyl, or substituted alkyl, of 1 to 24 carbons; halogen; -OR²¹; -NR²²R²³; -OM; a divalent linking group to another triazine; sulfonamide; substituted or unsubstituted alkylether of 1 to 20 carbons; polyethylene oxide of 2 to 40 carbons; -(OR²⁴)ₓR²⁵; -L²CR²⁶CH₂ or a polymer thereof;
- R¹⁵ and R¹⁶: independently represent sodium; potassium; ammonium; alkyl ammonium or substituted alkyl ammonium of 1 to 20 carbons; hydrogen; alkyl or substituted alkyl of 1 to 20 carbons ;
- R¹⁷ and R¹⁸: independently represent sodium; potassium; ammonium; hydrogen; alkyl ammonium or substituted alkyl ammonium of 1 to 20 carbons; alkyl or substituted alkyl or 1 to 20 carbons;
- R¹⁹ and R²⁰: independently represent sodium; potassium; hydrogen; ammonium; alkyl ammonium or substituted alkyl ammonium of 1 to 20 carbons; alkyl or substituted alkyl or 1 to 20 carbons ;
- R²¹: represents hydrogen; alkyl or substituted alkyl of 1 to 20 carbons; alkoxyalkyl or substituted alkoxyalkyl of 1 to 40 carbons; aryl or substituted aryl of 6 to 40 carbons; aralkyl or substituted aralkyl of 7 to 41 carbons; alkylthioether or substituted alkylthioether of 1 to 40 carbons;
- R²² and R²³: independently represent hydrogen; alkyl or substituted alkyl of 1 to 20 carbons; aryl or substituted aryl of 6 to 20 carbons; alkylether or substituted alkylether of 1 to 20 carbons; arylether or substituted arylether of 6 to 20 carbons; alkylthioether or substituted alkylthioether of 1 to 20 carbons; arylthioether or substituted arylthioether of 6 to 20 carbons; sulfonyl; alkylsulfonyl of 1 to 20 carbons;
- R²⁴: represents an ethylene or substituted ethylene;
- R²⁵: represents an alkyl or substituted alkyl of 1 to 20 carbons; an ether or substituted ether of 1 to 40 carbons;
- R²⁶: represents a hydrogen; alkyl or substituted alkyl of 1 to 24 carbons;
- L²: is a chemical linkage;
- M: is a counterion;
- x: is an integer from 1 to 24 ;
and a photographic element obtainable by this process.

### DETAILED DESCRIPTION OF THE INVENTION

Photographic elements of the present invention comprise at least one binder layer and at least one emulsion layer is crosslinked with at least one compound defined by Formula I and at least one compound defined by Formula II. Referring specifically to Formula I, Y¹ is an alkyl, or substituted alkyl, of 1 to 24 carbons; aryl, or substituted aryl, of 6 to 24 carbons; aralkyl or substituted aralkyl of 7 to 25 carbons; the atoms chosen from C, N, O, and S necessary to form a substituted or unsubstituted 5- or 6-membered ring; -L¹CR⁸CH₂, or a polymer thereof; -C(Y⁴)E; or E is an alkyl, or substituted alkyl, of 1 to 24 carbons; aryl, or substituted aryl, of 6 to 24 carbons; aralkyl or substituted aralkyl of 7 to 25 carbons; -OR⁹; -CN; the atoms chosen from C, N, O, and S necessary to form a substituted or unsubstituted 5- or 6-membered ring. L¹ is a linking group preferably chosen from a covalent chemical bond; alkyl, or substituted alkyl, of 1 to 20 carbons; aryl, or substituted aryl, of 6-24 carbons; aralkyl, or substituted aralkyl, of 7 to 25 carbons; carboxyl. Most preferably L¹ represents a chemical linkage; an alkyl, or substituted alkyl, of 1 to 3 carbons. R¹ is hydrogen; alkyl, or substituted alkyl, of 1 to 24 carbons; aryl, or substituted aryl, of 6 to 24 carbons; aralkyl, or substituted aralkyl, of 7 to 25 carbons; halogen; -OR¹⁰; halogen; nitro; carboxyl; mercapto; alklyamino or substituted alkylamino of 1 to 24 carbons; the atoms chosen from C, N, O and S necessary to from a 5- or 6-membered ring. Preferably R¹ represents hydrogen; alkyl, or substituted alkyl, of 1 to 3 carbons; aryl, or substituted aryl, of 6 to 10 carbons; aralkyl, or substituted aralkyl, of 7 to 11 carbons. Most preferably R¹ represents hydrogen; alkyl, or substituted alkyl, of 1 to 3 carbons. R² and R³ independently represent hydrogen; alkyl, or substituted alkyl, of 1 to 24 carbons; aryl, or substituted aryl, of 6 to 24 carbons; aralkyl, or substituted aralkyl, of 7 to 25 carbons. R² and R³ independently may represent, or be taken together to represent, the atoms C, N, O and S necessary to form a 5- or 6-membered ring. Preferably R² and R³ independently represent alkyl, or substituted alkyl, of 1 to 6 carbons; aryl, or substituted aryl, of 6 to 10 carbons; aralkyl, or substituted aralkyl, of 7 to 11 carbons; or taken together R² and R³ represent the atoms C, N and O necessary to form a 5- or 6-membered ring. Most preferably R² and R³ represent alkyl, or substituted alkyl, of 1 to 3 carbons or R² and R³ are taken together to represent the atoms C, N and O necessary to form a substituted or unsubstituted 5- or 6-membered ring. R⁴ and R⁵ independently represent hydrogen; alkyl, or substituted alkyl, of 1 to 24 carbons; aryl or substituted aryl of 6 to 24 carbons; aralkyl or substituted aralkyl of 7 to 25 carbons; nitro; carboxyl; mercapto; -OR¹¹; halogen; alkylamino or substituted alkylamino of 1 to 24 carbons; R⁴ and R⁵ independently may represent the atoms chosen from C, N, O, and S necessary to form a substituted or unsubstituted 5-or 6-member ring or R⁴ and R⁵ may be taken together to represent the atoms chosen from C, N, O, and S necessary to form a substituted or unsubstituted 5- or 6-membered ring. Preferably R⁴ and R⁵ independently represent hydrogen; alkyl, or unsubstituted alkyl, of 1 to 4 carbon atoms. X- is a counterion preferably chosen from the set consisting of halide, CF₃SO₃-, ClO₄-, BF4- and p-CH₃C₆H₄SO₃-. Y², Y³ and Y⁴ independently represent O or S. R⁶ and R⁷ independently represent hydrogen; alkyl, or substituted alkyl, of 1 to 24 carbons; aryl, or substituted aryl, of 6 to 24 carbons; aralkyl, or substituted aralkyl, of 7 to 25 carbons. R⁶ and R⁷ independently may represent, or be taken together to represent the atoms C, N, O and S necessary to form a substituted or unsubstituted 5- or 6-member ring. Preferably R⁶ and R⁷ independently represent alkyl, or substituted alkyl, of 1 to 6 carbons; aryl, or substituted aryl, of 6 to 10 carbons; aralkyl, or substituted aralkyl, of 7 to 11 carbons; taken together R⁶ and R⁷ may represent the atoms C, N and O necessary to form a substituted or unsubstituted 5- or 6-membered ring. Most preferably R⁶ and R⁷ represent alkyl, or substituted alkyl, of 1 to 3 carbons; or R⁶ and R⁷ are taken together to represent the atoms C, N and O necessary to form a substituted or unsubstituted 5- or 6-membered ring. R⁸ represents a hydrogen; an alkyl, or substituted alkyl, of 1 to 24 carbons; -C(O)R²⁸; -CN; aryl or substituted aryl of 6 to 24 carbons. R⁹ represents hydrogen; alkyl of substituted alkyl of 1 to 24 carbons; aryl of substituted aryl of 6 to 24 carbons. R¹⁰ and R¹¹ independently represent hydrogen; an alkyl, or substituted alkyl, of 1 to 5 carbons. R²⁸ represents hydrogen; alkyl or substituted alkyl of 1 to 24 carbons; alkoxy or substituted alkoxy of 1 to 24 carbons; amine; alkyl amine or substituted alkyl amine of 1 to 24 carbons.

Preferably in a compound of Formula I:
- Y²: represents O;
- R¹: is hydrogen; alkyl, or substituted alkyl, of 1 to 24 carbons; aryl, or substituted aryl, of 6 to 24 carbons; aralkyl, or substituted aralkyl, of 7 to 25 carbons; halogen;
- R² and R³: independently represent hydrogen; alkyl, or substituted alkyl, of 1 to 24 carbons; aryl, or substituted aryl, of 6 to 24 carbons; aralkyl, or substituted aralkyl, of 7 to 25 carbons; R² and R³ independently may represent, or be taken together to represent, the atoms chosen from C, N, O and S necessary to form a 5- or 6-membered ring;
- R² and R³: may be taken together to represent the atoms chosen from C, N, O, and S necessary to form a substituted or unsubstituted 5- or 6-membered ring;
- Y¹: is
wherein Y3 is O;
- R⁶ and R⁷: independently represent hydrogen; alkyl, or substituted alkyl, of 1 to 24 carbons; aryl, or substituted aryl, of 6 to 24 carbons; aralkyl, or substituted aralkyl, of 7 to 25 carbons; or the atoms chosen from C, N, O and S necessary to form a substituted or unsubstituted 5- or 6-membered ring; and
- R⁶ and R⁷: may be taken together to represent the atoms chosen from C, N, O and S necessary to form a substituted or unsubstituted 5- or 6-member ring.

In other preferred compounds of formula I
- Y¹: is an alkyl, or substituted alkyl, of 1 to 24 carbons; aryl, or substituted aryl, of 6 to 24 carbons; the atoms chosen from C, N, O, and S necessary to form a substituted or unsubstituted 5- or 6-membered ring; -L¹CR⁸CH₂, or a polymer thereof;
- L¹: is a linking group; and
- R⁸: represents a hydrogen; an alkyl, or substituted alkyl, of 1 to 3 carbons.

Consistent with terminology used in the art, the compound represented by: represents a vinyl imidazolium. The vinyl group of the vinyl imidazolium can be polymerized as known in the art to form a polymer. Preferably the vinyl group of the vinyl imidazolium can be polymerized with other substituted vinyl compounds to form a copolymer. Preferably the vinyl imidazole is a copolymer defined by: where R¹, R², R³, R⁴, R⁵, R⁸, L¹ and Y² correspond to the definition above for similiarly referenced groups. The subscript "p" represents the mole fraction of vinyl imidazolium monomer in the polymer and is preferably no more than 95% and more preferably no more than 50%. A and B independently represent copolymerized monomers. Preferably the monomers A and B are independently chosen from the set consisting of acrylic acid ester, methacrylic acid ester, acrylamide, styrene, styrene sulfonate, maleic anhydride, butadiene and vinyl chloride.

Referring specifically to Formula II. At least two of R¹², R¹³ and R¹⁴ are independently chosen from the groups represented by halogen, preferably Cl or Br; The most preferred group represented by R¹², R¹³ or R¹⁴ is chlorine or bromine. One of R¹², R¹³ or R¹⁴ may represent hydrogen; alkyl, or substituted alkyl, of 1 to 24 carbons, preferably 1 to 4 carbons; halogen; -OR²¹; -NR²²R²³; -OM; a linking group to another triazine; sulfonamide; substituted or unsubstituted alkyl ether of 1 to 20 carbons; polyethylene oxide of 2 to 40 carbons; -(OR²⁴)ₓR²⁵ where x is an integer from 1 to 24; -L²CR²⁶CH₂ or a polymer thereof. Preferably one substituent chosen from R¹², R¹³ or R¹⁴ is alkyl, of substituted alkyl, of 1 to 4 carbons; a halogen chosen from Cl and Br; -OR²¹; -NR²²R²³; -OM; a divalent linking group; sulfonamide; substituted or unsubstituted alkyl ether of 1 to 20 carbons; polyethylene oxide of 2 to 40 carbons; -(OR²⁴)ₓR²⁵ where x is an integer from 1 to 24; -L²CR²⁶CH₂ or a polymer thereof. Most preferrably one substituent chosen from R¹², R¹³ or R¹⁴ is -OM. R¹⁵ and R¹⁶ independently represent sodium; potassium; ammonium; alkyl ammonium or substituted alkyl ammonium of 1 to 20 carbons; hydrogen; alkyl or substituted alkyl of 1 to 20 carbons. Preferably R¹⁵ and R¹⁶ independently represent sodium; potassium; ammonium; alkylammonium or substituted alkylammonium of 1 to 4 carbons. R¹⁷ and R¹⁸ independently represent sodium; potassium; ammonium; hydrogen; alkyl ammonium or substituted alkyl ammonium of 1 to 20 carbons; alkyl or substituted alkyl or 1 to 20 carbons. Preferably R¹⁷ and R¹⁸ independently represent sodium; potassium; ammonium; or alkyl ammonium of 1 to 4 carbons. R¹⁹ and R²⁰ independently represent sodium; potassium; hydrogen; ammonium; alkyl ammonium or substituted alkyl ammonium of 1 to 20 carbons; alkyl or substituted alkyl or 1 to 20 carbons. Preferably R¹⁹ and R²⁰ independently represent sodium, potassium, ammonium, or alkyl ammonium of 1 to 4 carbons. R²¹ represents hydrogen, alkyl or substituted alkyl of 1 to 20 carbons; alkoxyalkyl or substituted alkoxyalkyl of 1 to 40 carbons; aryl or substituted aryl of 6 to 40 carbons; aralkyl or substituted aralkyl of 7 to 41 carbons; alkyl thioether or substituted alkyl thioether of 1 to 40 carbons. Preferably R²¹ represents hydrogen. R²² and R²³ independently represent hydrogen; alkyl or substituted alkyl of 1 to 20 carbons; aryl or substituted aryl of 6 to 20 carbons; alkylether or substituted alkylether of 1 to 20 carbons; arylether or substituted arylether of 6 to 20 carbons; alkylthioether or substituted alkylthioether of 1 to 20 carbons; arylthioether or substituted arylthioether of 6 to 20 carbons; sulfonyl; alkylsulfonyl of 1 to 20 carbons. Preferably R²² and R²³ independently represent hydrogen, sulfonyl, alkylsulfonyl of 1 to 4 carbons. R²⁴ represents an ethylene or substituted ethylene. Preferably R²⁴ represents ethylene or isopropylene. R²⁵ represents an alkyl or substituted alkyl of 1 to 20 carbons; an ether or substituted ether of 1 to 40 carbons. R²⁶ represents a hydrogen; alkyl or substituted alkyl of 1 to 24 carbons. Preferably R²⁶ represents a hydrogen or methyl. L² is a divalent chemical linkage preferably chosen from a chemical bond; alkylene or substituted alkylene of 1 to 20 carbons; arylene or substituted arylene of 6 to 24 carbons; aralkyl or substituted aralkyl of 7 to 25 carbons; or carbonyl. Preferably L² represents a chemical bond, alkylene or substituted alkylene of 1 to 10 carbons; arylene or substituted arylene of 6 to 10 carbons; aralkyl or substituted aralkyl of 7 to 12 carbons. M is a counterion. M is preferably chosen from sodium, potassium, lithium, calcium, barium, strontium, ammonium, or alkyl ammonium with 1 to 20 carbons. Most preferably M is chosen from sodium, potassium, ammonium, or alkyl ammonium of 1 to 20 carbons.

Preferably in a compound of Formula II at least two or R¹², R¹³ and R¹⁴ are halogen;
one of R¹², R^{13,} R¹⁴ is -OR²¹; NR²²R²³; -OM; a divalent linking group; sulfonamide;
- R²¹: represents hydrogen, alkyl or substituted alkyl of 1 to 20 carbons; alkoxyalkyl or substituted alkoxyalkyl of 1 to 40 carbons; aryl or substituted aryl of 6 to 10 carbons; aralkyl or substituted aralkyl of 7 to 41 carbons; alkyl thioether or substituted alkyl thioether of 1 to 40 carbons;
- R²² and R²³: independently represent hydrogen; alkyl or substituted alkyl or 1 to 20 carbons; aryl or substituted aryl of 6 to 20 carbons; alkylether or substituted alkyl ether of 1 to 20 carbons; aryl ether or substituted aryl ether of 6 to 20 carbons; alkyl thioether or substituted alkyl thioether of 1 to 20 carbons; aryl thioether or substituted aryl thioether of 6 to 20 carbons; sulfonyl; alkyl sulfonyl of 1 to 20 carbons;
- R²⁴: represents an ethyl or substituted ethyl;
- R²⁵: represents an alkyl of 1 to 20 carbons or an ether or 1 to 20 carbons;
- R²⁶: represents a hydrogen; alkyl or substituted alkyl of 1 to 24 carbons;
- L²: is a chemical linkage;
- M: is a counterion chosen from sodium, potassium, lithium, calcium, barium, strontium, ammonium, or alkyl ammonium with 1 to 20 carbons; and
- x: is an integer from 1 to 24.

Throughout this disclosure the group CH₂ = CR⁸- or CH₂ = CR²⁶- refers to the unpolymerized monomer. A polymer or copolymer formed by the polymerization or copolymerization of the vinyl group is also considered to be within the teachings of the present invention. The process of polymerization, or copolymerization, is well known in the art and includes specifically radical initiated polymerization.

The recitation "atoms chosen from C, N, O, and S necessary to from a 5- or 6-membered ring" or the equivalent thereof, refers to substituted or unsubstituted rings including but not limited to: the thiazole series; e.g. thiazole, 4-methylthiazole, 4-phenylthiazole, 5-methylthiazole, 5-phenylthiazole, 4,5-dimethylthiazole, 4,5-diphenylthiazole, 4-(2-thienyl)-thiazole;
the benzothiazole series; e.g., benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromobenzothiazole, 6-bromobenzothiazole, 4-phenylbenzothiazole, 5-phenylbenzothiazole, 4-methoxybenzothiazole, 5-methoxybenzothiazole, 6-methoxybenzothiazole, 5-iodobenzothiazole, 6-iodobenzothiazole, 4-ethoxybenzothiazole, 5-ethoxybenzothiazole, tetrahydrobenzothiazole, 5,6-dimethoxybenzothiazole, 5,6-dioxymethylenebenzothiazole, 5-hydroxybenzothiazole, 6-hydroxybenzothiazole;
the naphthothiazole series; e.g., naphtho[1,2]-thiazole, naphtho[2,1]thiazole, 5-methoxynaphtho-[2,1]-thiazole, 5-ethoxynaphtho[2,1]thiazole, 8-methoxynaphtho[1,2]thiazole, 7-methoxynaphtho[1,2]thiazole;
the thianaphtheno-7',6',4,5-thiazole series; e.g. 4'-methoxythianaphtheno-7',6',4,5,thiazole;
the oxazole series; e.g., 4-methyloxazole, 5-methyloxazole, 4-phenyloxazole, 4,5-diphenyloxazole, 4-ethyloxazole, 4,5-dimethyloxazole, 5-phenyioxazole;
the benzoxazole series; e.g., benzoxazole, 5-chlorobenzoxazole, 5-methylbenzoxazole, 5-phenylbenzoazole, 6-methylbenzoxazole, 5,6-dimethylbenzoxazole, 4,5-dimethylbenzoxazole, 5-methoxybenzoxazole, 5-ethoxybenzoxazole, 5-chlorobenzoxazole, 6-methoxybenzoxazole, 5-hydroxybenzoxazole, 6-hydroxybenzoxazole;
the naphthoxazole series, e.g., naphtho[1,2]oxazole, naphtho[2,1]oxazole;
the thiazoline series; e.g., thiazoline, 4-methylthiazoline;
the 2-quinoline series; e.g., quinoline, 3-methylquinoline, 5-methylquinoline, 7-methylquinoline, 8-methylquinoline, 6-chloroquinoline, 8-chloroquinoline, 6-methoxyquinoline, 6-ethoxyquinoline, 6-hydroxyquinoline, 8-hydroxyquinoline;
the 4-quinoline series; e.g., quinoline, 6-methoxyquinoline, 7-methoxyquinoline, 7-methylquinoline, 8-methylquinoline;
the 1-isoquinoline series; e.g., isoquinoline, 3,4-dihydroisoquinoline;
the 3-isoquinoline series; e.g., isoquinoline;
the benzimidazole series; e.g., 1,3-diethylbenzimidazole, 1-ethyl-3-phenylbenzimidazole;
the 3,3-dialkylindolenine series; e.g., 3,3-dimethylindoline, 3,3,5-trimethylindolenine, 3,3,7-trimethylindolenine;
the 2-pyridine series; e.g., pyridine, 5-methylpyridine; and the 4-pyridine series; e.g., pyridine;
the 3,3-dialkylbenz[e]indole series; e.g., 3,3-dimethylbenz[e]indole;
the tetrazole series: e.g., 1-phenyltetrazole, 1-methyltetrazole;
the triazole series: e.g., 1-phenyl-triazole, 1-methyltriazole;
the pyrimidine series: e.g., pyrimidine;
the thiadiazole series: e.g., 1,3,4-thiadiazole.

The terms "alkyl", "aryl", "aralkyl", "5- or 6-membered ring", and other groups refer to both unsubstituted and substituted groups unless specified to the contrary. Preferred substituents include halogen, nitro, carboxyl, hydroxyl, alkoxy, amine, thiol, amide, vinyl, sulfate, cyano, thioether, carboxylic acid, sulfonic acid, sulfato, and combination thereof.

Well known to the art is the advantage of using a surfactant to assist in coating a solution. Typically the surfactant is a separate entity

which is useful during coating and may be detrimental after coating is complete. By incorporating the surfactant into the chemical structure of the hardener the detrimental properties can be circumvented. A preferred embodiment of the present invention is realized when at least one of R¹, R², R³, R⁴, R⁵, R⁶, R⁷, R¹⁵, R¹⁶, R¹⁷, R¹⁸, R¹⁹, R²⁰, R²¹, R²², R²³ or one of the set consisting of R¹², R¹³ and R¹⁴ comprises a surfactant moiety incorporated into the chemical structure of the hardener. This allows a single compound to accomplish multiple task, namely, act as a coating aid during the coating process after which they act to crosslink the matrix as detailed above. Surfactant moieties which are known in the art include alkyls chains over 6 carbons, preferably 6 to 24 carbons; polyalkyleneoxide chains such as -(R²⁷O)ₘ-, wherein R²⁷ is ethylene, propylene or combinations thereof and m is an integer of 1 to 30; or combinations of alkylenes, and polyalkyleneoxides.

While not limited thereto, particularly preferred hardeners represented by Formula I are:

The structure of the imidazolium ring is known to exist with a delocalized charge. Comparable resonance structures can be drawn including:

While not limited thereto, particularly preferred hardeners represented by Formula II are:

The hardeners to be used in the present invention react rapidly with a hydrophilic colloid and therefore addition of the hardener to a solution containing hydrophilic colloid must be done with care. This is particularly important in the present invention since the compounds of Formula I and Formula II are incompatible as detailed previously. The hardeners to be used in the present invention are preferably added by injection into the solution supply line which transports coating solution from the holding tanks to the coater. The injection time is dependent on the coater configuration but the time between injection and coating must be sufficiently long to allow thorough mixing. It is also important that the time is not so long that crosslinking and decomposition begin to occur. An addition time of no more than approximately 5 minutes prior to coating is preferred and no more than 2 minutes is most preferred. Injection is accomplished by passing the coating solution past a "T" and adding a second hardener solution to the flow. After the "T" the two solutions are allowed to mix sufficiently.

The photographic element of the present invention can be coated onto a substrate with any method common to the art including but not limited to curtain coating, extrusion coating, slide-bead coating. Slide-bead coating is a preferred method.

Slide-bead coating is well known in the art to provide a means for supplying a flowing liquid layer or plurality of liquid layers down a slide surface to an efflux end, or lip, at which a liquid bridge, or bead, is formed in the gap between the lip and the moving substrate. The moving substrate carries away liquid from the liquid inventory in the bead in the same layered structure established on the slide. Exemplary examples include, for example, Russell, et.al., U. S. Patents 2,761,791 and 2,761,419.

The amount of hardener solution added depends on the degree of crosslinking desired. For use in a photographic emulsion the hardener solution is typically added in an amount sufficient to equal approximately 0.01 to 1.0 mmoles of Formula I per gram of hydrophilic colloid and approximately 0.01 to 1.0 mmoles of Formula II per gram of hydrophilic colloid. More preferred is approximately 0.02 to 0.30 mmoles of the hardener represented by Formula I per gram of hydrophilic colloid and approximately 0.02 to 0.30 mmoles of the hardener represented by Formula II per gram of hydrophilic colloid. The amount added may be different for different hydrophilic colloids.

The hardeners to be used in the present invention are most suitable for crosslinking a hydrophilic colloid layer. The hardeners to be used in the present invention are used for an emulsion layer containing hydrophilic colloid.

A photosensitive layer typically comprises silver halide dispersed in a hydrophilic colloid binder. The silver halide is optionally chemically and optionally spectrally sensitized as known in the art and the layer may contain other adjuvants such as dyes, stabilizers, development agents, color coupling agents, toners, surfactants.

An underlayer typically comprises a hydrophilic colloid layer with an optional dye dispersed therein. The overcoat is typically coated supra to the photosensitive layer as protection from, e.g., abrasion and may comprise dyes, surfactants, or other adjuvants as known in the art.

The term "hydrophilic colloid" or its homologues "gelatin" and "proteinaceous material" are used herein to refer to the protein substances which are derived from collagen. In the context of the present invention "hydrophilic colloid" also refers to substantially equivalent substances such as synthetic analogues of gelatin. Generally gelatin is classified as alkaline gelatin, acidic gelatin or enzymatic gelatin. Alkaline gelatin is obtained from the treatment of collagen with a base such as calcium hydroxide, for example. Acidic gelatin is that which is obtained from the treatment of collagen in acid such as, for example, hydrochloric acid and enzymatic gelatin is generated with a hydrolase treatment of collagen. The teachings of the present invention are not restricted to gelatin type or the molecular weight of the gelatin.

The film support for the emulsion layers used in the novel process may be any suitable transparent plastic. For example, the cellulosic supports, e.g. cellulose acetate, cellulose triacetate, cellulose mixed esters may be used. Polymerized vinyl compounds, e.g., copolymerized vinyl acetate and vinyl chloride, polystyrene, and polymerized acrylates may also be mentioned. Preferred films include those formed from the polyesterification product of a dicarboxylic acid and a dihydric alcohol made according to the teachings of Alles, U.S. Patent 2,779,684 and the patents referred to in the specification thereof. Other suitable supports are the polyethylene terephthalate/isophthalates of British Patent 766,290 and Canadian Patent 562,672 and those obtainable by condensing terephthalic acid and dimethyl terephthalate with propylene glycol, diethylene glycol, tetramethylene glycol or cyclohexane 1,4-dimethanol (hexahydro-p-xylene alcohol). The films of Bauer et al., U.S. Patent 3,052,543 may also be used. The above polyester films are particularly suitable because of their dimensional stability.

Meltpoint was measured by observing the melting temperature in 0.1 M NaOH for a hardened gelatin coating. Melt time was measured by observing the time, in minutes, required for the hardened layer to dissolve in a 1.5% NaOH solution at 50^{o}C. Water absorption was determined by weighing a dry 10cmx10cm film sample, submerging the sample for 30 minutes in an aqueous solution buffered to a pH of approximately 10.0 by a borate buffer, allowing the excess water on the surface to drain off of the film, and weighing the swollen film. Water absorption (WA) is defined as the weight gain per surface unit or as a percentage according the the equation:$\text{%WA =} \frac{\text{Wet weight - Dry weight (mg)}}{\text{Dry Weight}} \text{x 100}$

Wet gouge is a measure of the strength of the binder under processing conditions and is measured by dragging a stylus which increases force with distance over a film submerged in a mock developer solution comprising all ingredients except hydroquinone and phenidone. The wet gouge is then determined as the distance traversed by the stylus prior to destruction of the film surface. A larger distance indicates a stronger matrix.

### SYNTHESIS OF HARDENERS OF FORMULA I

### 1,3-bis-(dimethylcarbamoyl)-imidazolium chloride (I-14)

10.75 g (0.1 mole) dimethylcarbamoyl chloride are added dropwise with stirring to a solution of 6.8 g. (0.1 mole) imidazole and 11 g. triethylamine in 70 ml dry acetone. On warming, triethyl- ammonium chloride precipitates. After 5 hours standing at room temperature, the reaction mixture is filtered and 10.75 g. dimethyl- carbamoyl chloride is added again to the filtrate. After 2 days at room temperature, the crystalline product is filtered off, washed with acetone, and vacuum dried.

### 1,3-bis-(morpholinocarbonyl)-imidazolium chloride (I-20)

7.5 g. (0.05 mole) morpholino-4-carbonyl chloride are added to a solution of 3.4 g. (0.05 mole) imidazole and 5.5 g. triethylamine in 60 ml dry tetrahydrofuran. The mixture is stirred 30 minutes at 50^{o}C. The precipitated triethyl-ammonium chloride is filtered off. An additional 7.5 g morpholino-4-carbonyl chloride are added to the filtrate. After standing 2 days at room temperature, crystals of 1,3-bis-(morpholinocarbonyl)-imidazolium chloride separate, are filtered off, washed with ether and vacuum dried.

Standard organic reaction synthetic procedures can be employed as known in the art. While other synthetic procedures may be employed, the hardeners of Formula I were prepared in a consistent manner according to the following procedure. The appropriate N-substituted imidazol (0.2 mol) and the appropriate carbonyl chloride, or thiocarbaomyl chloride (0.2 mol) were dissolved in 100 ml. of acetone and refuxed for approximately 2 hrs. The reaction mixture was cooled to precipate the product which was then recovered by filtration. The filtrate was rinsed with acetone and dried in a dessicator at ambient conditions.

### 1-decyl-3-dimethylcarbamoylimidazolium bromide (I-1)

To 13.6 g (0.2 mole) of imidazole (Aldrich Chemical Co., Milwaukee, WI, 99%) and 20.2 g of triethylamine (Aldrich, 99%) in 100 ml dry acetone (Fisher Scientific Co., Pittsburgh, PA) in a magnetically stirred 250 ml round bottom flask under dry nitrogen was added 21.5 g (0.2 mole) dimethylcarbamyl chloride (Aldrich, 99%) dropwise over a 20 min. period from a side-arm pressure equalizing addition funnel. A white precipitate formed during the addition under conditions of mild exothermicity. The addition funnel was replaced with a reflux condensor and the reaction refluxed for a further one hour. After cooling to room temperature, the precipitate was isolated by Buchner filtration onto Wattman #1 paper, rinsed on the filter with acetone, and discarded. The combined filtrate and rinse acetone solution was divided into two equal parts, each containing 0.1 mole of 1-dimethylcarbamoylimidazole. To one of these parts was added 22.1 g (0.1 mole) of 1-bromodecane (Aldrich 98%) and the solution refluxed for seven hours under dry nitrogen. The acetone was evaporated at water aspirator vacuum in a rotoevaporator to the point where two layers formed. The upper layer contained largely unreacted bromodecane and the lower yielded 12 g (0.043 mole for a 21.4% theorical yield) of the imidazolium salt as a waxy solid upon cooling to 5^{o}C. The purity and identity of this product was confirmed by proton and carbon NMR in deuterium oxide solution.

### SYNTHETIC PROCEDURE FOR HARDENERS OF FORMULA II

### 2,4-dichloro-6-hydroxy-1,3,5-triazine, sodium salt (II-1)

1215 g of sodium phosphate tribasic was added to 70000 g. of water. The mixure was cooled to 24^{o}C and stirred until the sodium phosphate dissolved. 5000 g. of cyanuric chloride was added slowly. The pH was maintained between 8.0 and 9.5 with 1 N NaOH. After reaction is complete the pH is adjusted to approximately 7.8. The pH should not be allowed to drop below 7.7 at any time during the preparation or storage since rapid decomposition will commence.

### EXAMPLE 1

A photographic emulsion was prepared as known in the art. The emulsion comprised tabular silver halide grains and 70 grams of gelatin per mole of silver halide. The emulsion was coated on a subbed polyethylene terephthalate support to a silver coating weight of approximately 4.8 g/M². The combinations of hardeners listed in Table 1 were added either as a 2% solution (hardener I) or as a 10% solution (hardener II). The samples were held for approximately 1 week and analyzed yielding the results provided in Table 1.

**Table 1:**

| Physical Properties of Gelatin Layer Crosslinked with Hardeners of formulae I and II | | | | | |
|---|---|---|---|---|---|
| Hardener I | | Hardener II | | | |
| Hardener | Amount | Hardener | Amount | MT | |
| HCHO | 20.0 | - | - | 3 | Control |
| HCHO | 30.0 | - | - | 15 | Control |
| HCHO | 40.0 | - | - | 24 | Control |
| I-14 | 5.0 | - | - | 3 | Control |
| I-14 | 10.0 | - | - | 6 | Control |
| I-14 | 15.0 | - | - | 12 | Control |
| I-14 | 20.0 | - | - | 18 | Control |
| - | - | II-1 | 5.0 | 3 | Control |
| I-14 | 5.0 | II-1 | 5.0 | 6 | Inventive |
| I-14 | 10.0 | II-1 | 5.0 | 12 | Inventive |
| I-14 | 15.0 | II-1 | 5.0 | 15 | Inventive |
| I-14 | 20.0 | II-1 | 5.0 | 18 | Inventive |
| - | - | II-1 | 15.0 | 6 | Control |
| I-14 | 5.0 | II-1 | 15.0 | 9 | Inventive |
| I-14 | 10.0 | II-1 | 15.0 | 12 | Inventive |
| I-14 | 15.0 | II-1 | 15.0 | 15 | Inventive |
| I-14 | 20.0 | II-1 | 15.0 | 21 | Inventive |
| - | - | II-1 | 20.0 | 6 | Control |
| I-14 | 5.0 | II-1 | 20.0 | 9 | Inventive |
| I-14 | 10.0 | II-1 | 20.0 | 12 | Inventive |
| I-14 | 15.0 | II-1 | 20.0 | 18 | Inventive |
| I-14 | 20.0 | II-1 | 20.0 | 33 | Inventive |

Amount of hardener is listed as mmoles of hardener per 200 grams of gelatin. MT represents the melt time in minutes in 1.5 wt % NaOH at 50°C. The data demonstrates an increase in the crosslinking of the hydrophilic colloid binder as indicated by the increased MT observed with combinations of hardeners.

### EXAMPLE 2

An emulsion substantially similar to that used in Example 1 was prepared. Various hardener levels were added to individual aliquots as recorded in Table 2. The melt time (MT) and water absorption (WA mg/cm²) were measured after approximately 1 month and recorded in Table 2.

**Table 2:**

| Physical Properties of Gelatin Layer Crosslinked with Hardeners of formulae I and II | | | | | | |
|---|---|---|---|---|---|---|
| Hardener I | | Hardener II | | | | |
| Hardener | Amount | Hardener | Amount | MT | WA | |
| I-14 | 10.0 | - | - | 3 | .60 | Control |
| I-14 | 20.0 | - | - | 9 | .44 | Control |
| I-14 | 30.0 | - | - | 15 | .39 | Control |
| I-14 | 40.0 | - | - | 22 | .35 | Control |
| - | - | II-1 | 10.0 | 3 | .56 | Control |
| I-14 | 10.0 | II-1 | 10.0 | 9 | .42 | Inventive |
| I-14 | 20.0 | II-1 | 10.0 | 18 | .38 | Inventive |
| I-14 | 30.0 | II-1 | 10.0 | 24 | .35 | Inventive |
| I-14 | 40.0 | II-1 | 10.0 | 33 | .31 | Inventive |
| - | - | II-1 | 20.0 | 15 | .41 | Control |
| I-14 | 10.0 | II-1 | 20.0 | 18 | .38 | Inventive |
| I-14 | 20.0 | II-1 | 20.0 | 22 | .37 | Inventive |
| I-14 | 30.0 | II-1 | 20.0 | 28 | .33 | Inventive |
| I-14 | 40.0 | II-1 | 20.0 | 37 | .31 | Inventive |
| - | - | II-1 | 30.0 | 24 | .39 | Control |
| I-14 | 10.0 | II-1 | 30.0 | 25 | .37 | Inventive |
| I-14 | 20.0 | II-1 | 30.0 | 34 | .32 | Inventive |
| I-14 | 30.0 | II-1 | 30.0 | 34 | .32 | Inventive |
| I-14 | 40.0 | II-1 | 30.0 | 42 | .30 | Inventive |
| - | - | II-1 | 40.0 | 37 | .39 | Control |
| I-14 | 10.0 | II-1 | 40.0 | 33 | .35 | Inventive |
| I-14 | 20.0 | II-1 | 40.0 | 43 | .35 | Inventive |
| I-14 | 30.0 | II-1 | 40.0 | 46 | .34 | Inventive |
| I-14 | 40.0 | II-1 | 40.0 | 49 | .31 | Inventive |

The data of Table 3 indicates that the amount of water absorbed is lower when the combination of hardeners are used and the crosslinking is higher as indicated by the melt time.

### EXAMPLE 3 (Control)

An emulsion substantially similar to that described in Example 1 was prepared. The hardener levels recorded in Table 3. In Table 3 %WP represents the amount of water absorbed as a percentage of the total weight of the film; MT is the melt time in minutes; WG is wet gouge in grams.

**Table 3:**

| Physical Properties of Gelatin Layer Crosslinked with Hardeners of formulae II | | | | | | |
|---|---|---|---|---|---|---|
| Hardener I | | Hardener II | | | | |
| Hardener | Amount | Hardener | Amount | %WA | MT | WG |
| II-14 | 10.0 | II-1 | 4.1 | 14 | 7 | 4 |
| II-14 | 10.0 | - | - | 16 | 4 | 0 |
| - | - | II-1 | 4.1 | 17 | 3 | 0 |
| II-14 | 20.0 | II-1 | 8.2 | 13 | 19 | 3.5 |
| II-14 | 20.0 | - | - | 15 | 13 | 1.5 |
| - | - | II-1 | 8.2 | 15 | 3 | 0 |

In every case the film crosslinking is higher, as indicated by the MT or WG, and the water absorption is lower, as indicated by %WA when the combination of hardeners is employed.

The combined results of Examples 1-3 indicates that the additive effect of the hardeners can be appreciated without degradation of either.

## Claims

1. A process for forming a photographic element comprising the steps of:
forming at least one liquid photographic emulsion in at least one storage vessel wherein said liquid photographic emulsion comprises silver halide, hydrophilic colloid and a solvent;
transporting said liquid photographic emulsion to an interface region;
adding at least one compound I as defined below and at least one compound II as defined below;
mixing said liquid photographic emulsion with said compound I and said compound II thereby forming a coating solution;
transporting said coating solution to a coater;
coating said coating solution on a substrate thereby forming a liquid layer;
removing said solvent from said liquid layer to form a dry coated layer,
wherein the time between addition of the hardeners and coating is not so long that crosslinking and decomposition begin to occur;
compound I is a compound of Formula I: wherein:
Y¹ is an alkyl, or substituted alkyl, of 1 to 24 carbons; aryl, or substituted aryl, of 6 to 24 carbons; aralkyl or substituted aralkyl of 7 to 25 carbons; the atoms chosen from C, N, O, and S necessary to form a substituted or unsubstituted 5- or 6-membered ring; -L¹CR⁸CH₂, or a polymer thereof; -C(Y⁴)E; or
E is an alkyl, or substituted alkyl, of 1 to 24 carbons; aryl, or substituted aryl, of 6 to 24 carbons; aralkyl or substituted aralkyl of 7 to 25 carbons; -OR⁹; -CN; the atoms chosen from C, N, O, and S necessary to form a substituted or unsubstituted 5- or 6-membered ring;
L¹ is a linking group;
R¹ is hydrogen; alkyl, or substituted alkyl, of 1 to 24 carbons; aryl, or substituted aryl, of 6 to 24 carbons; aralkyl, or substituted aralkyl, of 7 to 25 carbons; -OR¹⁰; halogen; nitro, carboxyl, mercapto; alkylamino or substituted alkylamino of 1 to 24 carbons; the atoms chosen from C, N, O, and S necessary to form a substituted or unsubstituted 5- or 6-membered ring;
R² and R³ independently represent hydrogen; alkyl, or substituted alkyl, of 1 to 24 carbons; aryl, or substituted aryl, of 6 to 24 carbons; aralkyl, or substituted aralkyl, of 7 to 25 carbons; R² and R³ independently may represent, or be taken together to represent, the atoms chosen form C, N, O and S necessary to form a 5- or 6-membered ring;
R⁴ and R⁵ independently represent hydrogen; alkyl, or substituted alkyl, of 1 to 24 carbons; aryl or substituted aryl of 6 to 24 carbons; aralkyl or substituted aralkyl of 7 to 25 carbons; nitro; carboxyl; mercapto; -OR¹¹; halogen; alkylamino or substituted alkylamino of 1 to 24 carbons ;the atoms chosen from C, N, O, and S necessary to form a substituted or unsubstituted 5- or 6-membered ring;
R⁴ and R⁵ may be taken together to represent the atoms chosen from C, N, O, and S necessary to form a substituted or unsubstituted 5- or 6-membered ring;
X⁻ is a counterion;
Y², Y³ and Y⁴ independently represent O or S;
R⁶ and R⁷ independently represent hydrogen; alkyl, or substituted alkyl, of 1 to 24 carbons; aryl, or substituted aryl, of 6 to 24 carbons; aralkyl, or substituted aralkyl, of 7 to 25 carbons; the atoms chosen from C, N, O and S necessary to form a substituted or unsubstituted 5- or 6-membered ring;
R⁶ and R⁷ may be taken together to represent the atoms chosen from C, N, O and S necessary to form a substituted or unsubstituted 5- or 6-member ring;
R⁸ represents a hydrogen; an alkyl, or substituted alkyl, of 1 to 24 carbons; -C(O)R²⁸; -CN; aryl or substituted aryl of 6 to 24 carbons;
R⁹ represents hydrogen; alkyl or substituted alkyl of 1 to 24 carbons; aryl of substituted aryl of 6 to 24 carbons;
R¹⁰ and R¹¹ independently represent hydrogen, an alkyl, or substituted alkyl, of 1 to 5 carbons;
R²⁸ represents hydrogen; alkyl or substituted alkyl of 1 to 24 carbons; alkoxy or substituted alkoxy of 1 to 24 carbons; amine; alkylamine or substituted alkylamine of 1 to 24 carbons;
and compound II is a compound of Formula II: wherein:
at least two of R¹², R¹³ and R¹⁴ are independently chosen from the groups represented by halogen, preferably Cl or Br;
one of R¹², R¹³ or R¹⁴ may represent hydrogen; alkyl, or substituted alkyl, of 1 to 24 carbons; halogen; -OR²¹; -NR²²R²³; -OM; a divalent linking group to another triazine; sulfonamide; substituted or unsubstituted alkylether of 1 to 20 carbons; polyethylene oxide of 2 to 40 carbons; -(OR²⁴)ₓR²⁵; -L²CR²⁶CH₂ or a polymer thereof;
R¹⁵ and R¹⁶ independently represent sodium; potassium; ammonium; alkyl ammonium or substituted alkyl ammonium of 1 to 20 carbons; hydrogen; alkyl or substituted alkyl of 1 to 20 carbons;
R¹⁷ and R¹⁸ independently represent sodium; potassium; ammonium; hydrogen; alkyl ammonium or substituted alkyl ammonium of 1 to 20 carbons; alkyl or substituted alkyl or 1 to 20 carbons;
R¹⁹ and R²⁰ independently represent sodium; potassium; hydrogen; ammonium; alkyl ammonium or substituted alkyl ammonium of 1 to 20 carbons; alkyl or substituted alkyl or 1 to 20 carbons;
R²¹ represents hydrogen; alkyl or substituted alkyl of 1 to 20 carbons; alkoxyalkyl or substituted alkoxyalkyl of 1 to 40 carbons; aryl or substituted aryl of 6 to 40 carbons; aralkyl or substituted aralkyl of 7 to 41 carbons; alkylthioether or substituted alkylthioether of 1 to 40 carbons;
R²² and R²³ independently represent hydrogen; alkyl or substituted alkyl of 1 to 20 carbons; aryl or substituted aryl of 6 to 20 carbons; alkylether or substituted alkylether of 1 to 20 carbons; arylether or substituted arylether of 6 to 20 carbons; alkylthioether or substituted alkylthioether of 1 to 20 carbons; arylthioether or substituted arylthioether of 6 to 20 carbons; sulfonyl; alkylsulfonyl of 1 to 20 carbons;
R²⁴ represents an ethylene or substituted ethylene;
R²⁵ represents an alkyl or substituted alkyl of 1 to 20 carbons; an ether or substituted ether of 1 to 40 carbons;
R²⁶ represents a hydrogen; alkyl or substituted alkyl of 1 to 24 carbons;
L² is a chemical linkage;
M is a counterion;
X is an integer from 1 to 24.

2. The process recited in Claim 1 wherein in the compound of Formula I:
Y2 represents O;
R¹ is hydrogen; alkyl, or substituted alkyl, of 1 to 24 carbons; aryl, or substituted aryl, of 6 to 24 carbons; aralkyl, or substituted aralkyl, of 7 to 25 carbons; halogen;
R² and R³ independently represent hydrogen; alkyl, or substituted alkyl, of 1 to 24 carbons; aryl, or substituted aryl, of 6 to 24 carbons; aralkyl, or substituted aralkyl, of 7 to 25 carbons; R² and R³ independently may represent, or be taken together to represent, the atoms chosen from C, N, O and S necessary to form a 5- or 6-membered ring;
R² and R³ may be taken together to represent the atoms chosen from C, N, O, and S necessary to form a substituted or unsubstituted 5- or 6-membered ring;
Y¹ is
wherein Y3 is O;
R⁶ and R⁷ independently represent hydrogen; alkyl, or substituted alkyl, of 1 to 24 carbons; aryl, or substituted aryl, of 6 to 24 carbons; aralkyl, or substituted aralkyl, of 7 to 25 carbons; or the atoms chosen from C, N, O and S necessary to form a substituted or unsubstituted 5- or 6-membered ring;
R⁶ and R⁷ may be taken together to represent the atoms chosen from C, N, O and S necessary to form a substituted or unsubstituted 5- or 6-member ring.

3. The process recited in Claim 2 wherein the compound of Formula I is chosen from: and

4. The process recited in Claim 1 wherein in the compound of Formula I:
Y¹ is an alkyl, or substituted alkyl, of 1 to 24 carbons; aryl, or substituted aryl, of 6 to 24 carbons; the atoms chosen from C, N, O, and S necessary to form a substituted or unsubstituted 5- or 6-membered ring; -L¹CR⁸CH₂, or a polymer thereof;
L¹ is a linking group;
R⁸ represents a hydrogen; an alkyl, or substituted alkyl, of 1 to 3 carbons.

5. The process recited in Claim 4 wherein the compound of Formula I is chosen from: and

6. The process recited in Claim 1 wherein in the compound of Formula II at least two or R¹², R¹³ and R¹⁴ are halogen;
one of R¹², R¹³, R¹⁴ is -OR²¹; NR²²R²³; -OM; a divalent linking group; sulfonamide;
R²¹ represents hydrogen, alkyl or substituted alkyl of 1 to 20 carbons; alkoxyalkyl or substituted alkoxyalkyl of 1 to 40 carbons; aryl or substituted aryl of 6 to 10 carbons; aralkyl or substituted aralkyl of 7 to 41 carbons; alkyl thioether or substituted alkyl thioether of 1 to 40 carbons;
R²² and R²³ independently represent hydrogen; alkyl or substituted alkyl or 1 to 20 carbons; aryl or substituted aryl of 6 to 20 carbons; alkylether or substituted alkyl ether of 1 to 20 carbons; aryl ether or substituted aryl ether of 6 to 20 carbons; alkyl thioether or substituted alkyl thioether of 1 to 20 carbons; aryl thioether or substituted aryl thioether of 6 to 20 carbons; sulfonyl; alkyl sulfonyl of 1 to 20 carbons;
R²⁴ represents an ethyl or substituted ethyl;
R²⁵ represents an alkyl of 1 to 20 carbons or an ether or 1 to 20 carbons;
R²⁶ represents a hydrogen; alkyl or substituted alkyl of 1 to 24 carbons;
L² is a chemical linkage;
M is a counterion chosen from sodium, potassium, lithium, calcium, barium, strontium, ammonium, or alkyl ammonium with 1 to 20 carbons;
x is an integer from 1 to 24.

7. The process recited in Claim 6 wherein the compound of Formula II is chosen from:

8. A photographic element obtainable by the process of claims 1 to 7.

## Revendications

1. Procédé pour former un élément photographique, comprenant les étapes consistant à:
former au moins une émulsion photographique liquide dans au moins un récipient de stockage, dans lequel ladite émulsion photographique liquide comprend un halogénure d'argent, un colloïde hydrophile et un solvant;
transporter ladite émulsion photographique liquide à une région d'interface;
ajouter au moins un composé I tel que défini ci-dessous et au moins un composé II tel que défini ci-dessous;
mélanger ladite émulsion photographique liquide avec ledit composé I et avec ledit composé II pour ainsi former une solution de couchage;
transporter ladite solution de couchage à une coucheuse;
couler ladite solution de couchage sur un substrat pour ainsi former une couche liquide;
éliminer ledit solvant de ladite couche liquide pour former une couche sèche à l'état coulé,
dans lequel le laps de temps qui s'écoule entre l'addition des durcisseurs et le couchage n'est pas à ce point long qu'une réticulation et qu'une décomposition commencent à se manifester;
le composé I est un composé répondant à la formule I: dans laquelle:
Y¹ représente un groupe alkyle ou un groupe alkyle substitué contenant de 1 à 24 atomes de carbone; un groupe aryle ou un groupe aryle substitué contenant de 6 à 24 atomes de carbone; un groupe aralkyle ou un groupe aralkyle substitué contenant de 7 à 25 atomes de carbone; les atomes choisis parmi le groupe comprenant un atome de carbone, un atome d'azote, un atome d'oxygène et un atome de soufre, nécessaires pour former un noyau penta- ou hexagonal substitué ou non substitué; un groupe -L¹CR⁸CH₂ ou un polymère de ce dernier'; un groupe -C(Y⁴)E; ou encore un groupe répondant à la formule
E représente un groupe alkyle ou un groupe alkyle substitué contenant de 1 à 24 atomes de carbone; un groupe aryle ou un groupe aryle substitué contenant de 6 à 24 atomes de carbone; un groupe aralkyle ou un groupe aralkyle substitué contenant de 7 à 25 atomes de carbone; un groupe -OR⁹; un groupe -CN; les atomes choisis parmi le groupe comprenant un atome de carbone, un atome d'azote, un atome d'oxygène et un atome de soufre, nécessaires pour former un noyau penta- ou hexagonal substitué ou non substitué;
L¹ représente un groupe de liaison;
R¹ représente un atome d'hydrogène; un groupe alkyle ou un groupe alkyle substitué contenant de 1 à 24 atomes de carbone; un groupe aryle ou un groupe aryle substitué contenant de 6 à 24 atomes de carbone; un groupe aralkyle ou un groupe aralkyle substitué contenant de 7 à 25 atomes de carbone; un groupe -OR¹⁰; un atome d'halogène; un groupe nitro; un groupe carboxyle; un groupe mercapto; un groupe alkylamino ou un groupe alkylamino substitué contenant de 1 à 24 atomes de carbone; les atomes choisis parmi le groupe comprenant un atome de carbone, un atome d'azote, un atome d'oxygène et un atome de soufre, nécessaires pour former un noyau penta- ou hexagonal substitué ou non substitué;
R² et R³ représentent, indépendamment l'un de l'autre, un atome d'hydrogène; un groupe alkyle ou un groupe alkyle substitué contenant de 1 à 24 atomes de carbone; un groupe aryle ou un groupe aryle substitué contenant de 6 à 24 atomes de carbone; un groupe aralkyle ou un groupe aralkyle substitué contenant de 7 à 25 atomes de carbone; R² et R³ peuvent représenter indépendamment l'un de l'autre ou peuvent être pris ensemble pour représenter les atomes choisis parmi le groupe comprenant un atome de carbone, un atome d'azote, un atome d'oxygène et un atome de soufre, nécessaires pour former un noyau penta- ou hexagonal;
R⁴ et R⁵ représentent, indépendamment l'un de l'autre, un atome d'hydrogène; un groupe alkyle ou un groupe alkyle substitué contenant de 1 à 24 atomes de carbone; un groupe aryle ou un groupe aryle substitué contenant de 6 à 24 atomes de carbone; un groupe aralkyle ou un groupe aralkyle substitué contenant de 7 à 25 atomes de carbone; un groupe nitro; un groupe carboxyle; un groupe mercapto; un groupe -OR¹¹; un atome d'halogène; un groupe alkylamino ou un groupe alkylamino substitué contenant de 1 à 24 atomes de carbone; les atomes choisis parmi le groupe comprenant un atome de carbone, un atome d'azote, un atome d'oxygène et un atome de soufre, nécessaires pour former un noyau penta- ou hexagonal substitué ou non substitué;
R⁴ et R⁵ peuvent être pris ensemble pour représenter les atomes choisis parmi le groupe comprenant un atome de carbone, un atome d'azote, un atome d'oxygène et un atome de soufre, nécessaires pour former un noyau penta- ou hexagonal substitué ou non substitué;
X⁻ représente un ion complémentaire;
Y², Y³ et Y⁴ représentent, indépendamment l'un de l'autre, un atome d'oxygène ou un atome de soufre;
R⁶ et R⁷ représentent, indépendamment l'un de l'autre, un atome d'hydrogène; un groupe alkyle ou un groupe alkyle substitué contenant de 1 à 24 atomes de carbone; un groupe aryle ou un groupe aryle substitué contenant de 6 à 24 atomes de carbone; un groupe aralkyle ou un groupe aralkyle substitué contenant de 7 à 25 atomes de carbone; les atomes choisis parmi le groupe comprenant un atome de carbone, un atome d'azote, un atome d'oxygène et un atome de soufre, nécessaires pour former un noyau penta- ou hexagonal substitué ou non substitué;
R⁶ et R⁷ peuvent être pris ensemble pour représenter les atomes choisis parmi le groupe comprenant un atome de carbone, un atome d'azote, un atome d'oxygène et un atome de soufre, nécessaires pour former un noyau penta- ou hexagonal substitué ou non substitué;
R⁸ représente un atome d'hydrogène; un groupe alkyle ou un groupe alkyle substitué contenant de 1 à 24 atomes de carbone; un groupe -C(O)R²⁸; un groupe -CN; un groupe aryle ou un groupe aryle substitué contenant de 6 à 24 atomes de carbone;
R⁹ représente un atome d'hydrogène; un groupe alkyle ou un groupe alkyle substitué contenant de 1 à 24 atomes de carbone; un groupe aryle ou un groupe aryle substitué contenant de 6 à 24 atomes de carbone;
R¹⁰ et R¹¹ représentent, indépendamment l'un de l'autre, un atome d'hydrogène, un groupe alkyle ou un groupe alkyle substitué contenant de 1 à 5 atomes de carbone;
R²⁸ représente un atome d'hydrogène; un groupe alkyle ou un groupe alkyle substitué contenant de 1 à 24 atomes de carbone; un groupe alcoxy ou un groupe alcoxy substitué contenant de 1 à 24 atomes de carbone; un groupe amine; un groupe alkylamine ou un groupe alkylamine substitué contenant de 1 à 24 atomes de carbone;
et le composé II est un composé répondant à la formule II: dans laquelle:
au moins deux des radicaux R¹², R¹³ et R¹⁴ sont choisis, indépendamment l'un de l'autre, parmi le groupe comprenant des atomes d'halogène, de préférence un atome de chlore ou un atome de brome; les groupes
un des radicaux R¹², R¹³ ou R¹⁴ peut représenter un atome d'hydrogène; un groupe alkyle ou un groupe alkyle substitué contenant de 1 à 24 atomes de carbone; un atome d'halogène; un groupe -OR²¹; un groupe -NR²²R²³; un groupe -OM; un groupe de liaison divalent à une autre triazine; un groupe sulfonamide; un éther alkylique substitué ou non substitué contenant de 1 à 20 atomes de carbone; un oxyde de polyéthylène contenant de 2 à 40 atomes de carbone; un groupe -(OR²⁴)ₓR²⁵; un groupe -L²CR²⁶CH₂ ou un de ses polymères;
R¹⁵ et R¹⁶ représentent, indépendamment l'un de l'autre, le sodium; le potassium; l'ammonium; un groupe alkylammonium ou un groupe alkylammonium substitué contenant de 1 à 20 atomes de carbone; un atome d'hydrogène; un groupe alkyle ou un groupe alkyle substitué contenant de 1 à 20 atomes de carbone;
R¹⁷ et R¹⁸ représentent, indépendamment l'un de l'autre, le sodium; le potassium; l'ammonium; un atome d'hydrogène; un groupe alkylammonium ou un groupe alkylammonium substitué contenant de 1 à 20 atomes de carbone; un groupe alkyle ou un groupe alkyle substitué contenant de 1 à 20 atomes de carbone;
R¹⁹ et R²⁰ représentent, indépendamment l'un de l'autre, le sodium; le potassium; un atome d'hydrogène; l'ammonium; un groupe alkylammonium ou un groupe alkylammonium substitué contenant de 1 à 20 atomes de carbone; un groupe alkyle ou un groupe alkyle substitué contenant de 1 à 20 atomes de carbone;
R²¹ représente un atome d'hydrogène; un groupe alkyle ou un groupe alkyle substitué contenant de 1 à 20 atomes de carbone; un groupe alcoxyalkyle ou un groupe alcoxyalkyle substitué contenant de 1 à 40 atomes de carbone; un groupe aryle ou un groupe aryle substitué contenant de 6 à 40 atomes de carbone; un groupe aralkyle ou un groupe aralkyle substitué contenant de 7 à 41 atomes de carbone; un groupe thioéther alkylique ou un groupe thioéther alkylique substitué contenant de 1 à 40 atomes de carbone;
R²² et R²³ représentent, indépendamment l'un de l'autre, un atome d'hydrogène; un groupe alkyle ou un groupe alkyle substitué contenant de 1 à 20 atomes de carbone; un groupe aryle ou un groupe aryle substitué contenant de 6 à 20 atomes de carbone; un groupe éther alkylique ou un groupe éther alkylique substitué contenant de 1 à 20 atomes de carbone; un groupe éther arylique ou un groupe éther arylique substitué contenant de 6 à 20 atomes de carbone; un groupe thioéther alkylique ou un groupe thioéther alkylique substitué contenant de 1 à 20 atomes de carbone; un groupe thioéther arylique ou un groupe thioéther arylique substitué contenant de 6 à 20 atomes de carbone; un groupe sulfonyle; un groupe alkylsulfonyle contenant de 1 à 20 atomes de carbone;
R²⁴ représente un groupe éthylène ou un groupe éthylène substitué;
R²⁵ représente un groupe alkyle ou un groupe alkyle substitué contenant de 1 à 20 atomes de carbone; un groupe éther ou un groupe éther substitué contenant de 1 à 40 atomes de carbone;
R²⁶ représente un atome d'hydrogène; un groupe alkyle ou un groupe alkyle substitué contenant de 1 à 24 atomes de carbone;
L² représente une liaison chimique;
M représente un ion complémentaire;
X représente un entier de 1 à 24.

2. Procédé selon la revendication 1, dans lequel, dans le composé de formule I:
Y² représente un atome d'oxygène;
R¹ représente un atome d'hydrogène; un groupe alkyle ou un groupe alkyle substitué contenant de 1 à 24 atomes de carbone; un groupe aryle ou un groupe aryle substitué contenant de 6 à 24 atomes de carbone; un groupe aralkyle ou un groupe aralkyle substitué contenant de 7 à 25 atomes de carbone; un atome d'halogène;
R² et R³ représentent, indépendamment l'un de l'autre, un atome d'hydrogène; un groupe alkyle ou un groupe alkyle substitué contenant de 1 à 24 atomes de carbone; un groupe aryle ou un groupe aryle substitué contenant de 6 à 24 atomes de carbone; un groupe aralkyle ou un groupe aralkyle substitué contenant de 7 à 25 atomes de carbone; R² et R³ peuvent représenter indépendamment l'un de l'autre ou peuvent être pris ensemble pour représenter les atomes choisis parmi le groupe comprenant un atome de carbone, un atome d'azote, un atome d'oxygène et un atome de soufre, nécessaires pour former un noyau penta- ou hexagonal;
R² et R³ peuvent être pris ensemble pour représenter les atomes choisis parmi le groupe comprenant un atome de carbone, un atome d'azote, un atome d'oxygène et un atome de soufre, nécessaires pour former un noyau penta- ou hexagonal substitué ou non substitué;
Y¹ représente un groupe dans laquelle Y³ représente un atome d'oxygène;
R⁶ et R⁷ représentent, indépendamment l'un de l'autre, un atome d'hydrogène; un groupe alkyle ou un groupe alkyle substitué contenant de 1 à 24 atomes de carbone; un groupe aryle ou un groupe aryle substitué contenant de 6 à 24 atomes de carbone; un groupe aralkyle ou un groupe aralkyle substitué contenant de 7 à 25 atomes de carbone; ou encore représentent les atomes choisis parmi le groupe comprenant un atome de carbone, un atome d'azote, un atome d'oxygène et un atome de soufre, nécessaires pour former un noyau penta- ou hexagonal substitué ou non substitué;
R⁶ et R⁷ peuvent être pris ensemble pour représenter les atomes choisis parmi le groupe comprenant un atome de carbone, un atome d'azote, un atome d'oxygène et un atome de soufre, nécessaires pour former un noyau penta- ou hexagonal substitué ou non substitué.

3. Procédé selon la revendication 2, dans lequel le composé de formule I est choisi parmi le groupe comprenant: et

4. Procédé selon la revendication 1, dans lequel, dans le composé de formule I:
Y¹ représente un groupe alkyle ou un groupe alkyle substitué contenant de 1 à 24 atomes de carbone; un groupe aryle ou un groupe aryle substitué contenant de 6 à 24 atomes de carbone; les atomes choisis parmi le groupe comprenant un atome de carbone, un atome d'azote, un atome d'oxygène et un atome de soufre, nécessaires pour former un noyau penta- ou hexagonal substitué ou non substitué; un groupe -L¹CR⁸CH₂ ou un polymère de ce dernier;
L¹ représente un groupe de liaison;
R⁸ représente un atome d'hydrogène; un groupe alkyle ou un groupe alkyle substitué contenant de 1 à 3 atomes de carbone.

5. Procédé selon la revendication 4, dans lequel le composé de formule I est choisi parmi le groupe comprenant: et

6. Procédé selon la revendication 1, dans lequel, dans le composé de formule II, au moins deux des radicaux R¹², R¹³ et R¹⁴ représentent un atome d'halogène; un des radicaux R¹², R¹³, R¹⁴ représente un groupe -OR²¹; un groupe -NR²²R²³; un groupe -OM; un groupe de liaison divalent; un groupe sulfonamide;
R²¹ représente un atome d'hydrogène; un groupe alkyle ou un groupe alkyle substitué contenant de 1 à 20 atomes de carbone; un groupe alcoxyalkyle ou un groupe alcoxyalkyle substitué contenant de 1 à 40 atomes de carbone; un groupe aryle ou un groupe aryle substitué contenant de 6 à 10 atomes de carbone; un groupe aralkyle ou un groupe aralkyle substitué contenant de 7 à 41 atomes de carbone; un groupe thioéther alkylique ou un groupe thioéther alkylique substitué contenant de 1 à 40 atomes de carbone;
R²² et R²³ représentent, indépendamment l'un de l'autre, un atome d'hydrogène; un groupe alkyle ou un groupe alkyle substitué contenant de 1 à 20 atomes de carbone; un groupe aryle ou un groupe aryle substitué contenant de 6 à 20 atomes de carbone; un groupe éther alkylique ou un groupe éther alkylique substitué contenant de 1 à 20 atomes de carbone; un groupe éther arylique ou un groupe éther arylique substitué contenant de 6 à 20 atomes de carbone; un groupe thioéther alkylique ou un groupe thioéther alkylique substitué contenant de 1 à 20 atomes de carbone; un groupe thioéther arylique ou un groupe thioéther arylique substitué contenant de 6 à 20 atomes de carbone; un groupe sulfonyle; un groupe alkylsulfonyle contenant de 1 à 20 atomes de carbone;
R²⁴ représente un groupe éthyle ou un groupe éthyle substitué;
R²⁵ représente un groupe alkyle contenant de 1 à 20 atomes de carbone; un groupe éther contenant de 1 à 20 atomes de carbone;
R²⁶ représente un atome d'hydrogène; un groupe alkyle ou un groupe alkyle substitué contenant de 1 à 24 atomes de carbone;
L² représente une liaison chimique;
M représente un ion complémentaire choisi parmi le sodium, le potassium, le lithium, le calcium, le baryum, le strontium, l'ammonium ou un alkylammonium contenant de 1 à 20 atomes de carbone;
X représente un entier de 1 à 24.

7. Procédé selon la revendication 6, dans lequel le composé répondant à la formule II est choisi parmi le groupe comprenant:

8. Elément photographique que l'on obtient par le procédé selon les revendications 1 à 7.

## Patentansprüche

1. Ein Verfahren zur Bildung eines fotografischen Elements, das folgende Stufen umfaßt :
- die Bildung von wenigstens einer flüssigen fotografischen Emulsion in wenigstens einem Lagergefäß, wobei die flüssige fotografische Emulsion Silberhalogenid, hydrophiles Kolloid und ein Lösungsmittel enthält,
- die Beförderung der flüssigen fotografischen Emulsion zu einem Grenzbereich,
- die Zugabe von wenigstens einer nachstehend definierten Verbindung I und wenigstens einer nachstehend definierten Verbindung II,
- das Versetzen der flüssigen fotografischen Emulsion mit Verbindung I und Verbindung II zur Bildung einer Gießlösung,
- die Beförderung der Gießlösung zu einem Beschichtungsgerät,
- den Auftrag der Gießlösung auf ein Substrat, wodurch eine Flüssigkeitsschicht gebildet wird, und
- die Entfernung des Lösungsmittels aus der Flüssigkeitsschicht, wodurch eine trockene Schicht erhalten wird,
dadurch gekennzeichnet, daß die Zeit zwischen der Zugabe der Härter und dem Auftrag derart bemessen wird, daß keine Vernetzung und kein Abbau ausgelöst werden,
wobei Verbindung I Formel I entspricht : in der bedeuten :
Y¹ eine gegebenenfalls substituierte Alkylgruppe mit 1 bis 24 Kohlenstoffatomen, eine gegebenenfalls substituierte Arylgruppe mit 6 bis 24 Kohlenstoffatomen, eine gegebenenfalls substituierte Aralkylgruppe mit 7 bis 25 Kohlenstoffatomen, die zur Bildung eines gegebenenfalls substituierten fünf- oder sechsgliedrigen Ringes benötigten Atome aus der Gruppe bestehend aus C, N, O und S, -L¹CR⁸CH₂, oder ein Polymeres derselben, -C(Y⁴)E, oder
E eine gegebenenfalls substituierte Alkylgruppe mit 1 bis 24 Kohlenstoffatomen, eine gegebenenfalls substituierte Arylgruppe mit 6 bis 24 Kohlenstoffatomen, eine gegebenenfalls substituierte Aralkylgruppe mit 7 bis 25 Kohlenstoffatomen, -OR⁹, -CN, oder die zur Bildung eines gegebenenfalls substituierten fünf- oder sechsgliedrigen Ringes benötigten Atome aus der Gruppe bestehend aus C, N, O und S,
L¹ eine Verbindungsgruppe,
R¹ ein Wasserstoffatom, eine gegebenenfalls substituierte Alkylgruppe mit 1 bis 24 Kohlenstoffatomen, eine gegebenenfalls substituierte Arylgruppe mit 6 bis 24 Kohlenstoffatomen, eine gegebenenfalls substituierte Aralkylgruppe mit 7 bis 25 Kohlenstoffatomen, -OR¹⁰, ein Halogenatom, eine Nitrogruppe, eine Carboxylgruppe, eine Mercaptogruppe, eine gegebenenfalls substituierte Alkylaminogruppe mit 1 bis 24 Kohlenstoffatomen oder die zur Bildung eines gegebenenfalls substituierten fünf- oder sechsgliedrigen Ringes benötigten Atome aus der Gruppe bestehend aus C, N, O und S,
R² und R³ unabhängig voneinander ein Wasserstoffatom, eine gegebenenfalls substituierte Alkylgruppe mit 1 bis 24 Kohlenstoffatomen, eine gegebenenfalls substituierte Arylgruppe mit 6 bis 24 Kohlenstoffatomen, eine gegebenenfalls substituierte Aralkylgruppe mit 7 bis 25 Kohlenstoffatomen, oder R² und R³ unabhängig voneinander oder zusammen die zur Bildung eines fünf- oder sechsgliedrigen Ringes benötigten Atome aus der Gruppe bestehend aus C, N, O und S,
R⁴ und R⁵ unabhängig voneinander ein Wasserstoffatom, eine gegebenenfalls substituierte Alkylgruppe mit 1 bis 24 Kohlenstoffatomen, eine gegebenenfalls substituierte Arylgruppe mit 6 bis 24 Kohlenstoffatomen, eine gegebenenfalls substituierte Aralkylgruppe mit 7 bis 25 Kohlenstoffatomen, eine Nitrogruppe, eine Carboxylgruppe, eine Mercaptogruppe, -OR¹¹, ein Halogenatom, eine gegebenenfalls substituierte Alkylaminogruppe mit 1 bis 24 Kohlenstoffatomen oder die zur Bildung eines gegebenenfalls substituierten fünf- oder sechsgliedrigen Ringes benötigten Atome aus der Gruppe bestehend aus C, N, O und S,
oder R⁴ und R⁵ zusammen die zur Bildung eines gegebenenfalls substituierten fünf- oder sechsgliedrigen Ringes benötigten Atome aus der Gruppe bestehend aus C, N, O und S,
X⁻ ein Gegenion,
Y², Y³ und Y⁴ unabhängig voneinander O oder S,
R⁶ und R⁷ unabhängig voneinander ein Wasserstoffatom, eine gegebenenfalls substituierte Alkylgruppe mit 1 bis 24 Kohlenstoffatomen, eine gegebenenfalls substituierte Arylgruppe mit 6 bis 24 Kohlenstoffatomen, eine gegebenenfalls substituierte Aralkylgruppe mit 7 bis 25 Kohlenstoffatomen oder die zur Bildung eines gegebenenfalls substituierten fünf- oder sechsgliedrigen Ringes benötigten Atome aus der Gruppe bestehend aus C, N, O und S,
oder R⁶ und R⁷ zusammen die zur Bildung eines gegebenenfalls substituierten fünf- oder sechsgliedrigen Ringes benötigten Atome aus der Gruppe bestehend aus C, N, O und S,
R⁸ ein Wasserstoffatom, eine gegebenenfalls substituierte Alkylgruppe mit 1 bis 24 Kohlenstoffatomen, -C(O)R²⁸, -CN oder eine gegebenenfalls substituierte Arylgruppe mit 6 bis 24 Kohlenstoffatomen,
R⁹ ein Wasserstoffatom, eine gegebenenfalls substituierte Alkylgruppe mit 1 bis 24 Kohlenstoffatomen oder eine gegebenenfalls substituierte Arylgruppe mit 6 bis 24 Kohlenstoffatomen,
R¹⁰ und R¹¹ unabhängig voneinander ein Wasserstoffatom oder eine gegebenenfalls substituierte Alkylgruppe mit 1 bis 5 Kohlenstoffatomen,
R²⁸ ein Wasserstoffatom, eine gegebenenfalls substituierte Alkylgruppe mit 1 bis 24 Kohlenstoffatomen, eine gegebenenfalls substituierte Alkoxygruppe mit 1 bis 24 Kohlenstoffatomen, eine Aminogruppe oder eine gegebenenfalls substituierte Alkylaminogruppe mit 1 bis 24 Kohlenstoffatomen,
und Verbindung II Formel II entspricht : in der bedeuten :
wenigstens zwei Elemente der Reihe R¹², R¹³ und R¹⁴ unabhängig voneinander ein Halogenatom, vorzugsweise ein Chloratom oder Bromatom,
R¹², R¹³ oder R¹⁴ ein Wasserstoffatom, eine gegebenenfalls substituierte Alkylgruppe mit 1 bis 24 Kohlenstoffatomen, ein Halogenatom, -OR²¹, NR²²R²³, -OM, eine zweiwertige, an ein anderes Triazin gebundene Verbindungsgruppe, eine Sulfonamidgruppe, eine gegebenenfalls substituierte Alkylethergruppe mit 1 bis 20 Kohlenstoffatomen, eine Polyethylenoxidgruppe mit 2 bis 40 Kohlenstoffatomen, -(OR²⁴)_{X}R²⁵, -L²CR²⁶CH₂ oder ein Polymeres derselben,
R¹⁵ und R¹⁶ unabhängig voneinander eine Natriumgruppe, eine Kaliumgruppe, eine Ammoniumgruppe, eine gegebenenfalls substituierte Alkylammoniumgruppe mit 1 bis 20 Kohlenstoffatomen, ein Wasserstoffatom oder eine gegebenenfalls substituierte Alkylgruppe mit 1 bis 20 Kohlenstoffatomen,
R¹⁷ und R¹⁸ unabhängig voneinander eine Natriumgruppe, eine Kaliumgruppe, ein Wasserstoffatom, eine Ammoniumgruppe, ein Wasserstoffatom, eine gegebenenfalls substituierte Alkylammoniumgruppe mit 1 bis 20 Kohlenstoffatomen oder eine gegebenenfalls substituierte Alkylgruppe mit 1 bis 20 Kohlenstoffatomen,
R¹⁹ und R²⁰ unabhängig voneinander eine Natriumqruppe, eine Kaliumgruppe, ein Wasserstoffatom, eine Ammoniumgruppe, eine gegebenenfalls substituierte Alkylammoniumgruppe mit 1 bis 20 Kohlenstoffatomen oder eine gegebenenfalls substituierte Alkylgruppe mit 1 bis 20 Kohlenstoffatomen,
R²¹ ein Wasserstoffatom, eine gegebenenfalls substituierte Alkylgruppe mit 1 bis 20 Kohlenstoffatomen, eine gegebenenfalls substituierte Alkoxyalkylgruppe mit 1 bis 40 Kohlenstoffatomen, eine gegebenenfalls substituierte Arylgruppe mit 6 bis 40 Kohlenstoffatomen, eine gegebenenfalls substituierte Aralkylgruppe mit 7 bis 41 Kohlenstoffatomen oder eine gegebenenfalls substituierte Alkylthioethergruppe mit 1 bis 40 Kohlenstoffatomen,
R²² und R²³ unabhängig voneinander ein Wasserstoffatom, eine gegebenenfalls substituierte Alkylgruppe mit 1 bis 20 Kohlenstoffatomen, eine gegebenenfalls substituierte Arylgruppe mit 6 bis 20 Kohlenstoffatomen, eine gegebenenfalls substituierte Alkylethergruppe mit 1 bis 20 Kohlenstoffatomen, eine gegebenenfalls substituierte Arylethergruppe mit 6 bis 20 Kohlenstoffatomen, eine gegebenenfalls substituierte Alkylthioethergruppe mit 1 bis 20 Kohlenstoffatomen, eine gegebenenfalls substituierte Arylthioethergruppe mit 6 bis 20 Kohlenstoffatomen, eine Sulfonylgruppe oder eine Alkylsulfonylgruppe mit 1 bis 20 Kohlenstoffatomen,
R²⁴ eine gegebenenfalls substituierte Ethylengruppe,
R²⁵ eine gegebenenfalls substituierte Alkylgruppe mit 1 bis 20 Kohlenstoffatomen oder eine gegebenenfalls substituierte Ethergruppe mit 1 bis 40 Kohlenstoffatomen,
R²⁶ ein Wasserstoffatom oder eine gegebenenfalls substituierte Alkylgruppe mit 1 bis 24 Kohlenstoffatomen,
L² eine chemische Verbindungsgruppe,
M ein Gegenion, und
X eine ganze Zahl zwischen 1 und 24.

2. Verfahren nach Anspruch 1, dadurch gekennzeichnet, daß in der Verbindung der Formel I :
Y² ein Sauerstoffatom bedeutet,
R¹ ein Wasserstoffatom, eine gegebenenfalls substituierte Alkylgruppe mit 1 bis 24 Kohlenstoffatomen, eine gegebenenfalls substituierte Arylgruppe mit 6 bis 24 Kohlenstoffatomen, eine gegebenenfalls substituierte Aralkylgruppe mit 7 bis 25 Kohlenstoffatomen oder ein Halogenatom bedeutet,
R² und R³ unabhängig voneinander ein Wasserstoffatom, eine gegebenenfalls substituierte Alkylgruppe mit 1 bis 24 Kohlenstoffatomen, eine gegebenenfalls substituierte Arylgruppe mit 6 bis 24 Kohlenstoffatomen, eine gegebenenfalls substituierte Aralkylgruppe mit 7 bis 25 Kohlenstoffatomen, oder R² und R³ unabhängig voneinander oder zusammen die zur Bildung eines fünf- oder sechsgliedrigen Ringes benötigten Atome aus der Gruppe bestehend aus C, N, O und S bedeuten,
R² und R³ zusammen die zur Bildung eines gegebenenfalls substituierten fünf- oder sechsgliedrigen Ringes benötigten Atome aus der Gruppe bestehend aus C, N, O und S bedeuten können,
Y¹ bedeutet, in der bedeuten :
Y³ ein Sauerstoffatom,
R⁶ und R⁷ unabhängig voneinander ein Wasserstoffatom, eine gegebenenfalls substituierte Alkylgruppe mit 1 bis 24 Kohlenstoffatomen, eine gegebenenfalls substituierte Arylgruppe mit 6 bis 24 Kohlenstoffatomen, eine gegebenenfalls substituierte Aralkylgruppe mit 7 bis 25 Kohlenstoffatomen oder die zur Bildung eines gegebenenfalls substituierten fünf- oder sechsgliedrigen Ringes benötigten Atome aus der Gruppe bestehend aus C, N, O und S,
oder R⁶ und R⁷ zusammen die zur Bildung eines gegebenenfalls substituierten fünf- oder sechsgliedrigen Ringes benötigten Atome aus der Gruppe bestehend aus C, N, O und S.

3. Verfahren nach Anspruch 2, dadurch gekennzeichnet, daß die Verbindung der Formel I aus der nachstehenden Gruppe gewählt wird : und

4. Verfahren nach Anspruch 1, dadurch gekennzeichnet, daß in der Verbindung der Formel I :
Y¹ eine gegebenenfalls substituierte Alkylgruppe mit 1 bis 24 Kohlenstoffatomen, eine gegebenenfalls substituierte Arylgruppe mit 6 bis 24 Kohlenstoffatomen, die zur Bildung eines gegebenenfalls substituierten fünf- oder sechsgliedrigen Ringes benötigten Atome aus der Gruppe bestehend aus C, N, O und S, -L¹CR⁸CH₂, oder ein Polymeres derselben,
L¹ eine Verbindungsgruppe, und
R⁸ ein Wasserstoffatom oder eine gegebenenfalls substituierte Alkylgruppe mit 1 bis 3 Kohlenstoffatomen bedeuten.

5. Verfahren nach Anspruch 4, dadurch gekennzeichnet, daß die Verbindung der Formel I aus der nachstehenden Gruppe gewählt wird : and

6. Verfahren nach Anspruch 1, dadurch gekennzeichnet, daß in der Verbindung der Formel II :
wenigstens zwei Elemente der Reihe R¹², R¹³ und R¹⁴ ein Halogenatom bedeuten,
ein Element der Reihe R¹², R¹³ und R¹⁴ -OR²¹, NR²²R²³ oder -OM, eine zweiwertige Verbindungsgruppe oder eine Sulfonamidgruppe bedeutet,
R²¹ ein Wasserstoffatom, eine gegebenenfalls substituierte Alkylgruppe mit 1 bis 20 Kohlenstoffatomen, eine gegebenenfalls substituierte Alkoxyalkylgruppe mit 1 bis 40 Kohlenstoffatomen, eine gegebenenfalls substituierte Arylgruppe mit 6 bis 10 Kohlenstoffatomen, eine gegebenenfalls substituierte Aralkylgruppe mit 7 bis 41 Kohlenstoffatomen oder eine gegebenenfalls substituierte Alkylthioethergruppe mit 1 bis 40 Kohlenstoffatomen bedeutet,
R²² und R²³ unabhängig voneinander ein Wasserstoffatom, eine gegebenenfalls substituierte Alkylgruppe mit 1 bis 20 Kohlenstoffatomen, eine gegebenenfalls substituierte Arylgruppe mit 6 bis 20 Kohlenstoffatomen, eine gegebenenfalls substituierte Alkylethergruppe mit 1 bis 20 Kohlenstoffatomen, eine gegebenenfalls substituierte Arylethergruppe mit 6 bis 20 Kohlenstoffatomen, eine gegebenenfalls substituierte Alkylthioethergruppe mit 1 bis 20 Kohlenstoffatomen, eine gegebenenfalls substituierte Arylthioethergruppe mit 6 bis 20 Kohlenstoffatomen, eine Sulfonylgruppe oder eine Alkylsulfonylgruppe mit 1 bis 20 Kohlenstoffatomen bedeuten,
R²⁴ eine gegebenenfalls substituierte Ethylgruppe bedeutet,
R²⁵ eine Alkylgruppe mit 1 bis 20 Kohlenstoffatomen oder eine Ethergruppe mit 1 bis 20 Kohlenstoffatomen bedeutet,
R²⁶ ein Wasserstoffatom oder eine gegebenenfalls substituierte Alkylgruppe mit 1 bis 24 Kohlenstoffatomen bedeutet,
L² eine chemische Verbindungsgruppe bedeutet,
M ein Gegenion aus der Gruppe bestehend aus einer Natriumgruppe, Kaliumgruppe, Lithiumgruppe, Calciumgruppe, Bariumgruppe, Strontiumgruppe, Ammoniumgruppe und einer Alkylammoniumgruppe mit 1 bis 20 Kohlenstoffatomen bedeutet, und
X eine ganze Zahl zwischen 1 und 24 bedeutet.

7. Verfahren nach Anspruch 6, dadurch gekennzeichnet, daß die Verbindung der Formel II aus der nachstehenden Gruppe gewählt wird :

8. Ein durch das nach irgendeinem der Ansprüche 1 bis 7 definiertes Verfahren erhaltenes fotografisches Element.
